

## UNITED STATES PATENT OFFICE.

THOMAS MASON LUNAN, OF NEWARK, NEW JERSEY, ASSIGNOR TO THE CENTRAL STAMPING COMPANY, OF NEW YORK, A CORPORATION OF NEW YORK.

## MANUFACTURE OF ENAMELED WARE.

SPECIFICATION forming part of Letters Patent No. 758,325, dated April 26, 1904.

Application filed March 28, 1903. Serial No. 150,040. (No specimens.)

*To all whom it may concern:*

Be it known that I, THOMAS MASON LUNAN, a citizen of the United States, residing at Newark, county of Essex, State of New Jersey, have invented certain new and useful Improvements in the Manufacture of Enamelled Ware, of which the following is a specification.

My invention consists in a process of enameling metal ware.

10 The object of my invention is to produce enameled ware which will have a hard firm cohesive coating of attractive appearance and which owing to the acid character of the enamel will not be acted upon by acids or similar decomposing agents, as is the case where the enamel is of alkaline character.

To carry my invention into effect, I proceed as follows: The article to be enameled is first annealed and subsequently cleaned in any 20 well-known manner. After all the grease and dirt have been removed and the article dried it is dipped into a solution of potassium chlorate or sodium chlorate or other strong oxidizing solution. Potassium chlorate, as 25 is well-known, is one of the strongest oxidizing agents, and this body in the subsequent operation of baking to which the enameled article is subjected and even before breaks up according to the formula  $KClO_3 = KCl + 3O_2$ .

30 The nascent oxygen set free attacks the metal body of the article on which the enamel is to be applied, permeates it for a short distance, and forms a roughened surface, which forms an excellent point of attachment for the 35 enamel. The oxygen also converts all ferrous iron present in the composition of the enamel to ferric iron, and, further, raises all other metals present to a state of oxidation.

This step I consider of advantage. It may, 40 however, be entirely omitted. After the article to be enameled has been cleaned or after it has been subjected to treatment with the oxidizing solution, as above described, it is coated with an enamel of a distinctly acid nature, such as may be made by mixing various bodies—as, for instance, feldspar, silicic acid, calcium triphosphate, sodium carbonate, sodium tetraborate, and calcium fluorid with,

if it is desired, the addition of suitable coloring reagents—as, for instance, cobalt oxid—50 care being taken in compounding this coating to have the acidic part of the reagents in excess of the basic or alkaline part. This enamel after smelting is ground and brought to the desired consistency by the addition of clay or other suitable thickening reagent. The coating may be applied by dipping or otherwise. The article to be enameled may now be placed in the usual muffle and heated to set the enamel, or, preferably, in order to give the 60 enamel an attractive mottled or foliated appearance there is applied in the form of a spray or otherwise a solution of ammonium hydroxid or other non-metallic hydroxid, such as phenyl hydrozine. I do not limit myself, 65 however, to non-metallic hydroxids. The chemical action which takes place between the metallic bodies carried by the constituents of the enamel and the ammonium hydroxid are as follows for ferrous iron, ferric iron, and 70 aluminium:



These hydrated oxids form masses throughout the body of the enamel which greatly enhance the beauty of the article when finished. 80 After this treatment the article may be baked in a muffle in the usual manner. When the article is finished, it is covered with a beautifully-mottled and completely-oxidized enameled mass which by reason of its acid character will resist the action of all decomposing agents, in marked contrast to the behavior of ware coated with alkaline enamel, which, as is well known, is easily attacked by acids because of the excess of the basic radicals which 85 combine with the attacking acids forming their respective metallic salts, which in turn dissolve, thus allowing the enamel to easily disintegrate.

I make no claim in this application for the 95 article of manufacture resulting from the proc-

ess described, as the same has been made the subject of another application, Serial No. 195,229, filed February 25, 1904.

Having thus described my invention, I claim—

1. The herein-described process of enameling, which consists in coating the cleaned article with an enamel carrying metallic bodies and acid in character, then applying to said enameled surface a non-metallic hydroxid, and finally heating to flux and set the enamel.

2. The herein-described process of enameling, which consists in coating the cleaned article with an acid enamel of a character which will not attack the metal of which the article is made, and while still moist with a non-metallic hydroxid, and finally heating to flux and set the enamel.

3. The herein-described process of enameling which consists in coating the cleaned article with an acid enamel, and while still moist with a non-metallic hydroxid and finally heating to flux and set the enamel.

4. The herein-described process of enameling, which consists first in subjecting the cleaned article to the action of an oxidizing agent which will attack the metal of which the article is made, then applying a coating of acid enamel, then applying while the enamel is still moist a non-metallic hydroxid, and finally heating to flux and set the enamel.

5. The herein-described process of enameling which consists first, in subjecting the

cleaned article to the action of an oxidizing agent which will attack the metal, then applying a coating of acid enamel, then applying to said coating a non-metallic hydroxid, and finally heating to flux and set the enamel.

6. The herein-described process of enameling which consists first, in subjecting the cleaned article to the action of a solution of potassium chlorate, then applying a coating of acid enamel; then applying to said coating a non-metallic hydroxid, and finally heating to flux and set the enamel.

7. The herein-described process of enameling, which consists in applying to the cleaned article an acid enamel, then applying a suitable agent to precipitate the metallic body or bodies carried by said enamel, and finally heating to flux and set the enamel.

8. The herein-described process of producing a single-coat mottled enamel, which consists in coating the cleaned article with an acid enamel, and then applying a suitable agent to precipitate the metallic constituents of said enamel as masses, throughout the whole body of the enamel, and finally heating to flux and set the enamel.

In testimony whereof I affix my signature in the presence of two witnesses.

THOMAS MASON LUNAN.

Witnesses:

J. E. PEARSON,  
FRANK O'CONNOR.